

## UNITED STATES PATENT OFFICE

2,531,320

## RUST REMOVING

Thomas E. Burkhardt, Dayton, Ohio, assignor to  
General Motors Corporation, Dayton, Ohio, a  
corporation of Delaware

No Drawing. Original application September 25,  
1940, Serial No. 358,327. Divided and this ap-  
plication March 28, 1947, Serial No. 733,013

2 Claims. (Cl. 252—135)

1

This invention relates to a process for cleaning and polishing metal surfaces.

This application is a division of my copending application S. N. 358,327 filed September 25, 1940, Patent No. 2,428,141 issued September 30, 1947.

Heretofore, highly alkaline solutions such as sodium orthosilicate solutions have been used for electrolytically cleaning metal surfaces. It was found that such processes did not perform a sufficiently good job of cleaning and removing the oxide and scale. Also because of the high alkalinity of these solutions the workmen associated with these processes frequently suffered from skin diseases. These highly alkaline solutions were also objectionable since they attack the paint and enamel upon the parts to be cleaned. Furthermore, this and similar processes do not lend themselves readily to automatic conveyorized mechanized operation because the films that are built up during the transfer from one tank to another are not removed by such a cleaning process and become a source of trouble.

It is an object of my invention to provide a process of cleaning including removing oxide and scale from metal surfaces which is more thorough and which is less injurious to workmen employed thereon.

It is another object of my invention to provide a process of cleaning and/or removing oxide and scale from metal surfaces which will be effective when used in automatic conveyorized mechanized operation.

It is another object of my invention to provide a process of cleaning and/or removing oxide and scale from metal surfaces of articles in which paint and enamel on the articles cleaned will not be attacked.

It is still another object of my invention to provide a process of cleaning and/or removing oxide and scale from metal surfaces which will also polish the metal surfaces.

It is another object of my invention to provide a process for cleaning and polishing cast iron and steel surfaces which will also remove copper therefrom.

Further objects and advantages of the present invention will be apparent from the following description.

I have found by the use of phosphates in conjunction with other means, such as a wetting agent, or electric current, or a suitable acid or any combination of these, metal surfaces may be cleaned almost absolutely free of all traces of oxide and scale. Preferably my process employs an electrolyte formed of a low alkaline solution

2

having a pH value less than 10.5, preferably a low alkaline phosphate solution such as one selected from a group consisting of tetrasodium pyrophosphate, sodium metaphosphate and sodium hexametaphosphate. This electrolyte is kept at a fairly high temperature and the metallic surfaces to be cleaned are immersed in the electrolyte. The electrolyte is kept in agitation either by the movement of the metallic surfaces through the electrolyte or by some other suitable means. The process may be performed either anodically or cathodically, but preferably the current is passed from the metallic surfaces as anodes to a suitable cathode in contact with the electrolyte.

To obtain more rapid action a suitable wetting agent, a suitable acid or both may be included in the electrolyte. In some cases the process may be used non-electrolytically.

As an illustration there may be used an overhead conveyor for supporting articles to be electrolytically cleaned and polished. The articles for example, may include a sealed unit type of compressor having cast iron and steel surfaces to be cleaned, an aluminum tray, a copper plate and a cast iron reciprocating compressor. These are carried through an electrolyte contained in a tank of some suitable material, such as metal or earthen ware.

The electrolytic bath is provided with a suitable cathode of some suitable material, such as iron or nickel. This cathode is connected to a source of power for passing current from the articles as anodes through the electrolyte to the cathode.

The conveyor, when in operation, lowers the articles into the bath, connects them to the source of power, and moves the articles through the bath so as to cause agitation of the electrolytic bath adjacent the metal surface to be cleaned. Afterwards the articles are removed from the bath and carried into rinsing tanks and other such means. Preferably, the electrolyte comprises an aqueous solution of from 2 to 10 oz. per gallon of tetrasodium pyrophosphate. It has been found desirable to add a suitable wetting agent to the electrolyte. This increases the rapidity of the cleaning and/or removal of oxide and scale.

However, this is not absolutely necessary for the success of the process. Throughout the electrolytic treatment, the electrolyte is maintained at a temperature of between 180° and 210° F. or more. The current used is preferably at a potential of from 7 to 12 volts.

Copper, copper alloys, nickel, aluminum and similar metal surfaces may be thoroughly cleaned and polished by this process. When operated

anodically, this process not only thoroughly cleans the exposed metal surfaces but it also polishes them. This action is particularly noticeable upon copper and copper alloys. Where only traces of iron oxide and rust are present upon the iron and steel surfaces, these are also thoroughly cleaned and polished in this solution. Furthermore this process may also be used for removing immersion or electro-chemical deposits of copper on iron and steel at the same time the iron and steel parts are being cleaned anodically, since the copper is removed from the iron and steel as a part of their anodic cleaning process.

When more than traces of oxide coatings or rust are present upon iron and steel surfaces, it is desirable to use about 10 oz. per gallon of tetrasodium pyrophosphate in the electrolyte together with an amount sufficient to reduce the pH value to about 9 of an acid, such as acetic, citric, phosphoric, sulfuric, hydrochloric, nitric, and hydrofluoric acids. This solution may be used electrolytically or in a purely mechanical process. For still heavier oxide coatings, the pH value may be further lowered by the addition of more acid with a lower limit of 7. Likewise for lighter oxide coatings, less acid may be used with an upper limit of 10.5. Such a solution may be used for other metal surfaces.

Immediately following the electrolytic treatment, the articles are rinsed in clean cold running water with cold water sprays; following this, the articles are rinsed in clean soft hot running water at a temperature of 200° F. or more; finally, the articles are dried by air-blasts. After drying, the parts may be coated with an oil mixture where it is necessary to prevent rusting.

If desired, the electrolyte itself may be agitated by some other suitable means. Otherwise, the movement of the articles by the conveyor through the bath may be relied upon to provide sufficient agitation to remove any polarization or similar electrical effect. It is not necessary to use the conveyor or any such means for carrying out this process.

Sodium metaphosphate and sodium hexametaphosphate have somewhat similar properties as tetrasodium pyrophosphate and may be used in its place in substantially the same way. Other low alkaline phosphates may also be used. However, tetrasodium pyrophosphate is preferred.

I find that, in using this process, certain paints and black enamel, which may be upon the articles, are not attacked. Therefore, this process may be used for painted and enameled articles which have exposed metal surfaces requiring

cleaning. This is a particularly desirable advantage, since occasionally parts, after they have been painted or enameled, require reoperation and require cleaning of this type as a part of the reoperation procedure.

While it is desirable to maintain as set forth the specified temperatures, voltages and concentration, it is possible to use a solution of between 1 and 12 ozs. per gallon of tetrasodium pyrophosphate and to keep the temperature as low as 150° F. Also, voltages as low as 2 to 3 volts may be used for cleaning purposes, but for cleaning and polishing it is desirable to use at least 4 volts or more.

While the form of embodiment of the invention as herein disclosed, constitutes a preferred form, it is to be understood that other forms might be adopted, as may come within the scope of the claims which follow.

What is claimed is as follows:

1. The process of removing adherent rust from iron and steel surfaces which consists of immersing said surfaces for a sufficient length of time to remove the rust in an aqueous solution consisting essentially of about 10 oz. of tetrasodium pyrophosphate per gallon of water and an acid sufficient to reduce the pH value between 9 and 7.

2. The process of removing adherent rust from iron and steel surfaces which consists of immersing said surfaces for a sufficient length of time to remove the rust in an aqueous solution consisting essentially of an aqueous solution of tetrasodium pyrophosphate and an acid sufficient to reduce the pH value between 9 and 7.

THOMAS E. BURKHARDT.

#### REFERENCES CITED

The following references are of record in the file of this patent:

#### UNITED STATES PATENTS

| Number    | Name                   | Date           |
|-----------|------------------------|----------------|
| 1,572,848 | Porter et al. -----    | Feb. 9, 1926   |
| 2,093,927 | Preston -----          | Sept. 21, 1937 |
| 2,279,314 | Henderson et al. ----- | Apr. 14, 1942  |
| 2,304,850 | Rice -----             | Dec. 15, 1942  |

#### FOREIGN PATENTS

| Number  | Country             | Date           |
|---------|---------------------|----------------|
| 253,554 | Great Britain ----- | Sept. 14, 1927 |

#### OTHER REFERENCES

- Soap, November, 1938, pages 24, 25, 26 and 26A.  
Soap, August 1939, page 59.  
Soap, January 1939, pages 24, 25, 26 and 69.